

## UNITED STATES PATENT OFFICE

1,937,710

## BLEACHING ANIMAL FIBERS

Josef Müller, Weissenstein above the Drau, Austria, assignor, by mesne assignments, to E. I. du Pont de Nemours and Company, a corporation of Delaware

No Drawing. Application January 24, 1931,  
Serial No. 511,109, and in Austria January 31,  
1930

7 Claims. (Cl. 8—2)

This invention relates to bleaching animal fibers, such as hair, feathers, wool, and the like, with baths containing percompounds or compounds containing active oxygen. More particularly, the invention relates to bleaching stumps, clippings, or dead ends, of rabbit hair with solutions of compounds containing active oxygen, especially hydrogen peroxide.

Heretofore, bleaching of animal fibers, especially stumps of rabbit hair, has not been satisfactory. When using ordinary weakly alkaline hydrogen peroxide baths, a poor color and non-uniform hues were obtained. Furthermore, the loss of unused hydrogen peroxide by previous methods was high. The chief difficulties which have been encountered in bleaching rabbit hair have been due principally to the fact that the hair has previously been treated with nitric acid or mercuric nitrate or other nitrates for the purpose of felting the hair. Mercuric nitrate has chiefly been used for this purpose. When the treated or carotted hair is brought into contact with the hydrogen peroxide, especially if the carotting has been done with a mercury salt, various decomposition reactions occur which cause the bath to become very inefficient and produce a bad color. Also, the alkalinity of the baths previously used effected the property of the hair in an unsatisfactory manner.

The object of this invention is an improved bleach bath containing active oxygen compounds and its use in bleaching animal fiber, especially carotted rabbit hair and the like. A further object is a new hydrogen peroxide bleach bath and its use in bleaching animal fibers, which bath will bleach uniformly and thoroughly with a comparatively low consumption of active oxygen for the amount of bleaching action obtained, and which will give brighter hues than the usual alkaline solutions so used, to which ammonia and water glass and the like has been added. A further object of the invention is to retain the satisfactory quality of the material being treated, and in no case producing a hard feel under touch, such as that caused by alkaline baths.

It has now been found that the above objects, and others which may be evident from the description of my invention given below, can be attained by the use of a solution containing active oxygen, especially hydrogen peroxide, which is acid in reaction and which contains a dissolved aluminum salt. It has been found, for example, that a very good bleaching action

is obtained upon stumps of rabbit hairs, which have been carotted, by the use of an acid hydrogen peroxide solution to which has been added potassium alum. The following examples will serve to illustrate my invention.

1. Dark rabbit hair stumps for use in making hats were put into a bleaching solution which contained 1 per cent hydrogen peroxide and 1 per cent potassium alum. The reaction of this solution was weakly acid. The material was treated in this bath for twenty-four hours at 30° C. at the end of which time it had been made very much lighter in color without suffering any damage in the quality. The soft feel of the material remained just as it was before treating. The color effect was uniform and only 10 to 20% of the original hydrogen peroxide was used.

When the raw material of this example was bleached in the usual alkaline bath, the bleaching effect was not nearly so good and the feel of the material was hard. In most cases, the samples in such a bath had a very poor color. Furthermore, the amount of peroxide necessary, or used, was considerably higher than that used in the above example.

2. Dark bed feathers were put into a bath containing 5 per cent of hydrogen peroxide in addition to 0.25% of alum and 0.25% of sodium-aluminum chloride. The solution reacted weakly acid. After treating the material twenty-four hours at 30° C. it was much brighter in color and had not experienced any deterioration of quality.

If one bleaches the material of this example in the usual alkaline solution, the amount of active oxygen compound will need to be about 50% higher and the bleach will be no better. An alkaline bath used under these conditions also gives indications of having been destroyed.

The above described acid bleach baths containing dissolved aluminum salts have been used for bleaching of all kinds of human hair as well as wool yarn. It has been found that the quality of these products is not damaged, whereas the properties of the same material, when employing the usual alkaline hydrogen peroxide baths, is always harmed to a marked degree. Although in some instances, the extent of the bleach may be weaker than is the case when using an alkaline bleach, nevertheless, if one uses the baths of this invention a considerably better quality of bleached material is obtained.

Instead of potassium alum, other soluble

aluminum salts such as aluminum chloride, aluminum sulphate, sodium alum, sodium-aluminum chloride and other complex salts of aluminum can be used. Instead of bleaching with hydrogen peroxide in acid solution, other compounds giving off active oxygen can be used in an acid bath.

This invention is not to be confused with that of German Patent #313,541 wherein is described bleaching textile material with sodium perborate in a bleach bath to which has been added free alkali and soap and such small quantities of aluminum salt, aluminum hydroxide or aluminate, that no separation occurs. Furthermore, the present invention, describing the use of soluble compounds of aluminum, differs fundamentally from that method described in Austrian Patent #65,734, wherein insoluble compounds of aluminum or tin are added to the bleach bath.

What I claim is:

1. Process of bleaching animal fibers which comprises treating the material to be bleached in an acid solution containing a soluble aluminum salt and a compound capable of liberating active oxygen.

2. Process of bleaching animal fibers which comprises treating the material to be bleached in an acid solution containing a soluble aluminum salt and hydrogen peroxide.

3. Process of bleaching carotted rabbit hair which comprises treating the hair in an acid solution containing a soluble aluminum salt and a compound capable of liberating active oxygen.

4. Process of bleaching carotted rabbit hair which comprises treating the hair in an acid solution containing a soluble aluminum salt hydrogen peroxide.

5. Process of bleaching rabbit hair previously carotted with mercury compound which comprises treating the hair in an acid solution containing dissolved potassium alum and hydrogen peroxide.

6. A bleach bath having an acid reaction and containing a soluble aluminum salt and a compound which is capable of liberating active oxygen.

7. A bleach bath having an acid reaction and containing a dissolved alum and hydrogen peroxide.

JOSEF MÜLLER.

20

105

35

110

40

115

45

120

50

125

55

130

60

135

65

140

70

145

150